

## UNITED STATES PATENT OFFICE

2,448,571

SIZED ORGANIC DERIVATIVE OF  
CELLULOSE YARNRalph H. Balch and Irma G. McCormick, Cum-  
berland, Md., assignors to Celanese Corporation  
of America, a corporation of DelawareNo Drawing. Application July 18, 1945,  
Serial No. 605,848

3 Claims. (Cl. 117—139.5)

1

This invention relates to an improved sizing composition comprising casein, and relates more particularly to the sizing of yarns with said sizing composition.

An object of this invention is the provision of an improved sizing composition containing casein which may be employed for the sizing of yarns prior to weaving or other textile operations.

Another object of this invention is the provision of a sizing composition comprising casein plasticized with a nitrogenous base such as triethanolamine, and containing an organic ester of phosphoric acid.

A further object of this invention is to provide an improved sizing composition especially adapted for the sizing of yarns having a basis of cellulose acetate or other organic derivative of cellulose.

Other objects of this invention will appear from the following detailed description.

Yarns, especially synthetic yarns, are usually treated with a size to enable them to withstand the textile operations of weaving and the like. Usually such sizes contain gelatin as a base. However, gelatin is at times difficult to obtain and, furthermore, when employed for sizes, requires the use of softening agents such as vegetable oils, sulfonated oils, sulfonated waxes, as well as penetrants and surface active agents. The use of casein instead of gelatin in regular size formulations does not produce a satisfactory size, since none of the various oils and softeners heretofore used in gelatin sizes has any appreciable softening or plasticizing effect on casein, so that when warps are sized with compositions containing casein and such oils and softeners, there occur undesirable effects such as frost or tear marks.

We have now found that an excellent sizing composition having a basis of casein may be obtained if there is incorporated with the casein not only a nitrogenous base such as an alkyloamine but also an organic ester of phosphoric acid. Both the nitrogenous base and the phosphoric acid ester act as softening and plasticizing agents for the casein and produce an excellent dispersion of the casein when incorporated in the aqueous medium by means of which the size is applied to the yarns.

The novel sizing compositions produced in accordance with our invention may be applied to any yarns whether made of continuous filaments or spun from fibers of staple length. These yarns may comprise natural fibers, or they may comprise synthetic fibers having a basis of cel-

2

lulose acetate or other organic derivative of cellulose, or filaments or fibers of regenerated cellulose made by the viscose or cuprammonium process or by the saponification of yarns having a basis of a cellulose ester. These sizing compositions may also be applied to yarns having a basis of a synthetic linear polyamide condensation product, such as polymerized hexamethylene adipamide or yarns having a basis of polymerized vinyl compounds. Especially valuable results are obtained when these improved sizing compositions are employed in the sizing of yarns made of or containing organic acid esters of cellulose, such as cellulose acetate, cellulose propionate, cellulose butyrate, cellulose acetate-propionate and cellulose acetate-butyrate, as well as cellulose ethers, such as ethyl cellulose or benzyl cellulose.

The casein employed in preparing our novel sizing composition is preferably raw casein obtained from skim milk and coagulated by means of acid, salts, electrodialysis, or by any other known method of preparing casein in the desired form.

25 The alkyloamine employed in accordance with our invention may be triethanolamine, diethanolamine, trimethanolamine, tripropionalmine or mixtures of these amines. However, we preferably employ commercial triethanolamine, which 30 may contain small quantities of diethanolamine and monoethanolamine. Organic esters of phosphoric acid which we have found to be suitable are, for example, triethyl phosphate, triphenyl phosphate, tributyl phosphate or tricresyl phosphate. However, triethyl phosphate has been 35 found to yield the most advantageous results.

The several components of our novel sizing composition are preferably present in the following amounts: from 75 to 85% by weight of casein, 15 to 20% by weight of the alkyloamine and 3.5 to 6% by weight of the organic phosphoric acid ester. The sizing composition is normally applied in such an amount of water as to give a solution of the desired consistency, 45 the amount of water varying with the degree of sizing necessary to produce the desired result in subsequent weaving or other textile operations.

While the organic phosphoric acid esters are 50 capable of exerting a plasticizing action on cellulose acetate or organic derivative of cellulose materials, we have found that the use of our novel sizing composition has no adverse effect on said materials even where the cellulose acetate or other organic derivative of cellulose textile ma-

terials sized with these compositions are stored for a considerable period of time with the size remaining thereon. There is no loss of strength or elongation in the sized cellulose acetate materials. The presence of the organic phosphoric acid esters in fact imparts considerably more flexibility to the yarns and greatly increases the weaving efficiency, producing a product free from frost with substantially reduced end breakage due to the size.

In order further to illustrate our invention, but without being limited thereto, the following example is given:

*Example*

The size is made of the following components:

|                                   | Pounds |
|-----------------------------------|--------|
| Casein (raw) -----                | 50     |
| Triethanolamine -----             | 10     |
| Triethyl phosphate -----          | 3      |
| Water, q. s. to make 100 gallons. |        |

The triethanolamine is dissolved in the water at room temperature and the casein is then added slowly with agitation over the course of 30 minutes. The triethyl phosphate is then added and the solution heated to 150° F. and held at this temperature for 10 minutes. It is then strained through cheese cloth and is then ready for use. The sizing composition prepared in this manner has a pH of 7.0. The size is applied to a warp made of continuous filaments of cellulose acetate at 150° F. in the usual apparatus employed for sizing warps. When this warp is woven into a satin fabric, the latter is produced with excellent weaving efficiency, the end breakage comprising only 3.9 ends per 100 yards.

When the cellulose acetate material carrying our novel sizing composition is stored for three weeks at 65% relative humidity and at a temperature of 70° F., or even at a temperature of 100 to 120° F., the initial properties are wholly retained without loss of strength or elongation and no coalescence of the filaments takes place.

It is to be understood that the foregoing de-

tailed description is given merely by way of illustration and that many variations may be made without departing from the spirit of our invention.

Having described our invention, what we desire to secure by Letters Patent is:

1. A textile yarn of cellulose acetate sized with a composition comprising about 79% by weight of casein, about 16% of triethanolamine and about 5% of triethyl phosphate.

2. A textile yarn having a basis of an organic derivative of cellulose and sized with a composition comprising 75 to 85% by weight of casein, 15 to 20% of an alkyloamine and 3.5 to 6% of an organic ester of phosphoric acid selected from the group consisting of tri-ethyl phosphate, tri-phenyl phosphate, tri-butyl phosphate and tri-cresyl phosphate.

3. A textile yarn having a basis of cellulose acetate and sized with a composition comprising 75 to 85% by weight of casein, 15 to 20% of an alkyloamine and 3.5 to 6% of an organic ester of phosphoric acid selected from the group consisting of tri-ethyl phosphate, tri-phenyl phosphate, tri-butyl phosphate and tri-cresyl phosphate.

RALPH H. BALCH,  
IRMA G. McCORMICK.

**REFERENCES CITED**

The following references are of record in the file of this patent:

**UNITED STATES PATENTS**

| 35 | Number    | Name                  | Date          |
|----|-----------|-----------------------|---------------|
|    | 2,312,469 | Freund -----          | Mar. 2, 1943  |
|    | 2,310,795 | La Piana et al. ----- | Feb. 9, 1943  |
|    | 2,262,771 | La Piana et al. ----- | Nov. 18, 1941 |
| 40 | 2,201,992 | Dreyfus et al. -----  | May 28, 1940  |
|    | 2,191,654 | Haon -----            | Feb. 27, 1940 |

**FOREIGN PATENTS**

| Number  | Country             | Date          |
|---------|---------------------|---------------|
| 550,838 | Great Britain ----- | Jan. 27, 1943 |